



US006280274B1

(12) **United States Patent**  
Hofmann et al.

(10) **Patent No.:** US 6,280,274 B1  
(45) **Date of Patent:** \*Aug. 28, 2001

(54) **FIBER SPACERS IN LARGE AREA VACUUM DISPLAYS AND METHOD FOR MANUFACTURE**

3,875,442 4/1975 Wasa et al. .  
3,979,621 9/1976 Yates .

(List continued on next page.)

(75) Inventors: **James J. Hofmann; Jason B. Elledge**, both of Boise, ID (US)

FOREIGN PATENT DOCUMENTS

(73) Assignee: **Micron Technology, Inc.**, Boise, ID (US)

690472 A1 3/1996 (EP) .  
2-165540 6/1990 (JP) .

(\*) Notice: Subject to any disclaimer, the term of this patent is extended or adjusted under 35 U.S.C. 154(b) by 0 days.

OTHER PUBLICATIONS

This patent is subject to a terminal disclaimer.

Hashiguchi, Mimur and Hiroyuki, "Fabrication and Emission Characteristics of Polycrystalline Silicon Field Emitters," Jpn. J. Appl. Phys. vol. 34 (1995).

(21) Appl. No.: **09/652,290**

(22) Filed: **Aug. 31, 2000**

Itoh, S., Niizuma, T., and Yokoyama, M., "Influence of Various Gases on the Emission of Field Emitter Arrays," Futaba Corporation (2 pages).

Levy, F., and Meyer, R., "Phosphors for Full-Color Microtips Fluorescent Displays," Conference Record of the 1991 International Display Research Conference, pp. 20-23.

**Related U.S. Application Data**

*Primary Examiner*—Kenneth J. Ramsey

(63) Continuation of application No. 09/414,862, filed on Oct. 12, 1999, now Pat. No. 6,155,900.

(74) *Attorney, Agent, or Firm*—Traskbrill, P.C.

(51) **Int. Cl. 7** ..... **H01J 9/00**

**ABSTRACT**

(52) **U.S. Cl.** ..... **445/24; 313/495**

A process for fabricating high-aspect ratio support structures comprising: creating a rectangular fiber bundle by stacking selectively etchable glass strands having rectangular cross-sections; slicing the fiber bundle into rectangular tiles; adhering the tiles to an electrode plate of an evacuated display; and selectively removing glass strands, thereby creating support structures.

(58) **Field of Search** ..... **445/24; 313/25, 313/495; 65/31, 42, 408, 411, 429**

**48 Claims, 7 Drawing Sheets**

(56) **References Cited**

**U.S. PATENT DOCUMENTS**

3,424,909 1/1969 Rougeot .  
3,812,559 5/1974 Spindt et al. .



## U.S. PATENT DOCUMENTS

|           |         |                    |           |           |                            |
|-----------|---------|--------------------|-----------|-----------|----------------------------|
| 3,990,874 | 11/1976 | Schulman .         | 5,342,477 | 8/1994    | Cathey .                   |
| 4,091,305 | 5/1978  | Poley et al. .     | 5,342,737 | 8/1994    | Georger, Jr. et al. .      |
| 4,183,125 | 1/1980  | Meyer et al. .     | 5,347,292 | 9/1994    | Ge et al. .                |
| 4,292,092 | 9/1981  | Hanak .            | 5,371,433 | 12/1994   | Home et al. .              |
| 4,451,759 | 5/1984  | Heynisch .         | 5,374,868 | 12/1994   | Tjaden et al. .            |
| 4,705,205 | 11/1987 | Allen et al. .     | 5,391,259 | 2/1995    | Cathey et al. .            |
| 4,749,840 | 6/1988  | Piwczyk .          | 5,413,513 | 5/1995    | Home et al. .              |
| 4,874,461 | 10/1989 | Sato et al. .      | 5,445,550 | 8/1995    | Xie et al. .               |
| 4,892,592 | 1/1990  | Dickson et al. .   | 5,448,131 | 9/1995    | Taylor et al. .            |
| 4,923,421 | 5/1990  | Brodie et al. .    | 5,449,970 | 9/1995    | Kumar et al. .             |
| 4,940,916 | 7/1990  | Borel et al. .     | 5,486,126 | 1/1996    | Cathey et al. .            |
| 4,973,378 | 11/1990 | Lee et al. .       | 5,561,343 | 10/1996   | Lowe .                     |
| 5,070,282 | 12/1991 | Epsztein .         | 5,621,272 | 4/1997    | Levine et al. .            |
| 5,136,764 | 8/1992  | Vasquez .          | 5,634,585 | 6/1997    | Stansbury .                |
| 5,151,061 | 9/1992  | Sandhu .           | 5,648,698 | 7/1997    | Makishima et al. .         |
| 5,205,770 | 4/1993  | Lowrey et al. .    | 5,708,325 | 1/1998    | Anderson et al. .          |
| 5,209,688 | 5/1993  | Nishigaki et al. . | 5,717,287 | 2/1998    | Amrine et al. .            |
| 5,229,691 | 7/1993  | Shichao et al. .   | 5,795,206 | 8/1998    | Cathey et al. .            |
| 5,232,549 | 8/1993  | Cathey et al. .    | 5,811,927 | 9/1998    | Anderson et al. .          |
| 5,324,602 | 6/1994  | Inada et al. .     | 5,989,090 | 11/1999   | Perrin et al. .            |
| 5,329,207 | 7/1994  | Cathey et al. .    | 6,155,900 | * 12/2000 | Hofmann et al. .... 445/24 |

\* cited by examiner



FIG. 1



FIG. 2A



FIG. 2B



FIG. 2C



FIG. 3



FIG. 4



FIG. 5



FIG. 6A



FIG. 6B



FIG. 6C

**FIBER SPACERS IN LARGE AREA VACUUM  
DISPLAYS AND METHOD FOR  
MANUFACTURE**

**CROSS-REFERENCE TO RELATED  
APPLICATION**

This application is a continuation of application Ser. No. 09/414,862, filed Oct. 12, 1999, now U.S. Pat. No. 6,155,900, issued Dec. 5, 2000.

**GOVERNMENTAL RIGHTS**

This invention was made with Government support under Contract No. DABT63-93-C-0025 awarded by Advanced Research Projects Agency (ARPA). The Government has certain rights in this invention.

**BACKGROUND OF THE INVENTION**

**1. Field of the Invention**

This invention relates to flat panel display devices and, more particularly, to processes for creating fiber spacer structures which provide support against the atmospheric pressure on the flat panel display without impairing the resolution of the image.

**2. State of the Art**

In flat panel displays of the field emission type, an evacuated cavity is maintained between the cathode electron-emitting surface and its corresponding anode display face. Since there is a relatively high voltage differential between the cathode emitting surface and the display screen, it is important to prevent catastrophic electrical breakdown between them. At the same time, the narrow spacing between the plates is necessary for structural thinness and to obtain high image resolution. Spacer structures incorporated between the display face and the baseplate perform these functions.

In order to be effective, spacer structures must possess certain characteristics. They must have sufficient non-conductivity to prevent catastrophic electrical breakdown between the cathode array and the anode. This is necessary because of both the relatively close inter-electrode spacing (which may be on the order of 200  $\mu$ m), and relatively high inter-electrode voltage differential (which may be on the order of 300 or more volts).

Further, the supports must be strong enough to prevent the flat panel display from collapsing under atmospheric pressure. Stability under electron bombardment is also important, since electrons will be generated at each of the pixels. The spacers must also withstand "bake-out" temperatures of around 400° C. used in forming the high vacuum between the faceplate and baseplate of the display.

For optimum screen resolution, the spacer structures must be almost perfectly aligned to array topography. They must be of sufficiently small cross-sectional area so as to be invisible during display operation. Hence, cylindrical spacers must have diameters no greater than about 50 microns. A single cylindrical lead oxide silicate glass column, having a diameter of 25 microns and a height of 200 microns, will have a buckle load of about  $2.67 \times 10^{-2}$  newtons. Buckle loads, of course, will decrease as height is increased with no corresponding increase in diameter.

It is also of note that a cylindrical spacer having a diameter  $d$  will have a buckle load that is only about 18% greater than that of a spacer of square cross-section and a diagonal  $d$ , although the cylindrical spacer has a cross-sectional area about 57% greater than the spacer of square cross section.

Known methods for spacer fabrication using screen-printing, stencil printing, or glass balls do not provide a spacer having a sufficiently high aspect ratio. The spacers formed by these methods either cannot support the high voltages, or interfere with the display image. Other methods which employ the etching of deposited materials suffer from slow throughput (i.e., time length of fabrication), slow etch rates, and etch mask degradation. The use of lithographically defined photoactive organic compound results in the formation of spacers, which are incompatible with the high vacuum conditions, and elevated temperatures characteristic in the manufacture of field emission displays (FED).

Accordingly, there is a need for a high aspect ratio spacer structure for use in a FED, and an efficient method of manufacturing a FED with such a spacer.

**BRIEF SUMMARY OF THE INVENTION**

A process for fabricating high-aspect ratio support structures is provided. The process comprises creating a rectangular fiber bundle of glass strands, wherein contiguous groups of glass strands form a pattern. The pattern can be of a variety of shapes, including a cross, tee, I-beam, rail, or bracket. The fiber bundle is sliced into "tiles" and adhered to an electrode plate of an evacuated display.

The fiber bundle is comprised of groups of selectively etchable glass strands, which may or may not be coated with a resistive material. The glass strands are preferably square in cross-section, and are therefore stackable. The etchable and nonetchable strands are stacked in a desired pattern in the bundle; the bundle is drawn to thereby increase its length and decrease its diameter, while maintaining its shape and pattern. Several bundles are then stacked, and drawn into a fiber boule. The fiber boule is sliced into rectangular tiles. Adhesive is deposited on the electrode plate of the vacuum display to hold the tiles in the desired locations, and the tiles disposed about the display plate. Some of the glass fibers are then selectively removed, thereby creating support structures.

In an alternative embodiment of the present invention, a process for forming spacers useful in large area displays is disclosed. The process comprises forming rectangular bundles comprising fiber strands held together with a binder; slicing the bundles into rectangular slices, adhering the slices onto an electrode plate of the display; and removing the binder. The ends of the glass fibers may be polished, and the binder near the ends of the glass fibers etched back. The binder is then removed, thereby creating spacers.

One advantage of this method of stacking fibers in a pattern and forming boules therefrom is that collimated spacers are made in an accurate, repeatable pattern, not easily attainable when other shapes, such as round fibers are utilized. This reduces the cost of manufacturing the panel, as well as the weight of the panel. The use of such spacers enables the sintering of thin panel glass substrates, while holding off the forces due to atmospheric pressure. This technique will also result in high aspect ratio spacers, so higher resolution can be attained without having the output image adversely affected by the presence of spacers. This technique also increases the chances that the fiber strand is orderly and regularly distributed in the glass boule. The evenly collimated distribution is maintained throughout the spacer forming process, thereby improving the yield in the percentage of fibers adhering onto the glue dots.

**BRIEF DESCRIPTION OF THE SEVERAL  
VIEWS OF THE DRAWINGS**

The present invention will be better understood from reading the following description of nonlimitative

embodiments, with reference to the attached drawings, wherein below:

FIG. 1 is a schematic cross-section of a representative pixel of a field emission display comprising a faceplate with a phosphor screen, vacuum sealed to a baseplate which is supported by the spacers formed according to the process of the present invention;

FIG. 2A is a schematic cross-section of a fiber bundle fabricated according to the process of the present invention;

FIG. 2B is a schematic cross-section of a group of fiber bundles of FIG. 2A arranged in a boule, which is drawn to an intermediate size, according to the process of the present invention;

FIG. 2C is a schematic cross-section of the boule of fiber bundles of FIG. 2B, which has been drawn to a smaller size and sliced, according to the process of the present invention;

FIG. 3 is a schematic side-view of a slice of the boule of FIG. 2C, fabricated according to the process of the present invention;

FIG. 4 is a schematic cross-section of the electrode plate of a flat panel display without the slices of FIG. 3 disposed thereon;

FIG. 5 is a schematic cross-section of an electrode plate of a flat panel display with the slices of FIG. 3 disposed thereon;

FIGS. 6A-C are schematic cross-sections of a spacer support structure, fabricated according to the process of the present invention;

FIG. 6A is a spacer support structure comprising columns disposed about the electrode plate, according to the process of the present invention;

FIG. 6B is a spacer support structure comprising a rail support disposed about the electrode plate, according to an alternative embodiment of the process of the present invention; and

FIG. 6C is a spacer support structure comprising a cross-rail support structure disposed about the electrode plate, according to another alternative embodiment of the process of the present invention.

#### DETAILED DESCRIPTION OF THE INVENTION

Referring to FIG. 1, a representative field emission display employing a display segment 22 is depicted. Each display segment 22 is capable of displaying a pixel of information. A black matrix 25 (FIG. 4), or grille, surrounds the segments for improving the display contrast. Gate 15 serves as a grid structure for applying an electrical field potential to its respective cathode 13. When a voltage differential, through source 20, is applied between the cathode 13 and the gate 15, a stream of electrons 17 is emitted toward a phosphor coated screen or faceplate 16. A dielectric insulating layer 14 is deposited on the conductive cathode 13.

Disposed between faceplate 16 and baseplate 21 are located spacer support structures 18, which function to support the atmospheric pressure that exists between them as a result of the vacuum.

The process of the present invention provides a method for fabricating high aspect ratio support structures to function as spacer support structures 18 through the use of stackable glass fiber strands, which have a rectangular or substantially square cross-section.

Various aspects of using fibers for spacer structures are described in U.S. Pat. No. 5,486,126 entitled, Spacers for

Large Area Displays and U.S. Pat. No. 5,795,206 entitled, Fiber Spacers in Large Area Vacuum Displays and Method for Manufacture of Same, which are commonly owned with the present invention. These patents are hereby incorporated by reference as if set forth in their entirety.

The preferred manufacturing process, according to the present invention, starts with fibers or strands of a non-etchable glass, such as, but not limited to, potash rubidium lead. The non-etchable glass preferably does not etch in hydrochloric acid and has significant etch resistance to aqueous hydrofluoric acid.

The etchable spacer support structures 18 are comprised of glass which has a high lead content, preferably greater than 40%. PbO added to the glass in sufficient amounts will make it soluble in HCl or other acids. The viscosity-temperature curve can be adjusted by varying the other components of the glass, such as, for example,  $Na_2O$ ,  $CaO_2$ ,  $Al_2O_3$ , and other materials. Since the completed and assembled display is later "baked out," the coefficient of thermal expansion of the glass strands should be close to that of a substrate material 11 which is used for the display face 16 and/or baseplate 21.

The fiber strands, used in the present invention, may employ a high resistance coating which allow a very slight bleed off of stray electrons to occur over time. This will prevent a destructive arc over. Highly resistive silicon is one example of a thin coating that is useful on the fiber strands. Such a coating is applied by techniques commonly known in the art, such as chemical vapor deposition (CVD) of an organic-metal material or sputtering or evaporating a thin layer of carbon onto the silicon.

The starting non-etchable glass strand is preferably square or rectangular in cross-section. Commercially available fibers have widths from about 0.18" to 0.25" which are much too large for use as a spacer support. This width is substantially reduced through the process of the present invention, so that the width of the final glass strand is in the range of 0.001" to 0.002".

As depicted in FIG. 2A, the non-etchable glass strands or fibers 18A are assembled in a pattern with etchable glass strands or fibers 18B to thereby form a mixed glass assembly 28 of a generally contiguous group of glass strands or fibers 18A, 18B. Small gaps will occur if glass strands or fibers 18A are dislodged from the mixed glass assembly 28 as a result of the manufacturing process. Since the glass strands or fibers 18A, 18B are rectangular in shape, they are relatively easy to stack in patterns. The mixed glass assembly 28 will also be rectangular, and preferably, square in cross-section. The shape of the final spacer structure will be comprised of a pattern formed by the cross-sections of a plurality of the contiguous rectangular non-etchable glass strands or fibers 18A.

The mixed glass assembly 28 is thermally drawn down to an intermediate size. The result of this drawing step is a single-fiber unit cell or bundle 28' having a diameter of approximately 0.125". The drawing step is preferably performed in a drawing tower. The single-fiber unit cell 28', formed from the mixed glass assembly 28, has a reduced cross-section and increased length.

Several steps of glass technology are applied to transform the single-fiber unit cells 28' into a glass boule 38, as will be described herein. Such a boule 38 is comprised of up to 2000 glass fibers. FIG. 2B depicts the square or rectangular arrangement of stacked single-fiber unit cells 28'. The single-fiber unit cells 28' are tacked together in an oven (at a temperature above 100° C. below the glass softening temperature) so that the shape is maintained.

As depicted in FIG. 2C, the boule 38 or stack of single-fiber unit cells is redrawn down to the final desired dimension. Each group of contiguous non-etchable fibers 18A is surrounded by a pattern that is selectively etchable with respect to it. The fibers 18A are regularly distributed in a collimated, i.e., parallel and evenly spaced manner within the single-fiber unit cells 28'. The outer shape is substantially rectangular, and the cross-sections are rectangular or square.

After drawing, there is an adherence between the glass strands of the single-fiber unit cells 28'. This may be sufficient to hold the strands, in some cases. However, in other cases, the stability of the boule 38 is further enhanced by placing the drawn boule of fibers in a mold and fusing the strands under pressure, whereby a sintered, solid boule 38 is created. The boule 38 is made in a press exerting mechanical pressure on the outside of the stacked single-fiber unit cells. Appropriate sintering temperature is applied, as well as vacuum of about  $10^{-3}$  Torr for removing gas from the interstices between the fibers. Alternatively, a vacuum is not applied during sintering. Acceptable sintering parameters include 300–500° C.  $\pm 20^\circ$  C. for several hours (between about 4–12 hours) with adequate time for annealing and cool down (about 6–12 hours for annealing and cool down). The time varies depending on thickness and pressure.

Alternatively, the glass fibers can be coated with a binder material to assist in maintaining them in the desired pattern. A temporary binder may be applied to individual fibers 18A, 18B prior to bundling, or to several fibers 18A, 18B at a time in a mixed glass assembly 28 or in close proximity, to provide spacing between fibers 18A, 18B.

However, in the preferred embodiment, no binder material is employed. Since the fibers 18A, 18B have a rectangular or substantially square cross-section, they are readily stacked in a pattern and formed into single-fiber unit cells or bundles 28' and/or boules 38.

FIGS. 2B and 2C depict the boule 38 which is sliced, on average, at about 0.015" to 0.020" with a wafer saw. The thickness of the slice will determine whether the cross-section of the rail is rectangular or square. Depending on how well the previous steps were carried out, there may be some unevenness in height among the strands. Hence, planarizing may be done at this point. Chemical-mechanical planarization can be used to even out the fibers. This step also polishes the fiber ends flat and parallel.

Once the slices or tiles 29 of fibers have been created, they are attached to one of the electrode plates 16, 21 of the evacuated display. Referring now to FIG. 4, dots of adhesive 26 are provided at the sites where the spacer support structures 18 are to be located. Some examples of adhesives include, but are not limited to, potassium silicates and sodium silicates, which are alkaline solutions that bond glass really well when dried. Alternatively epoxies can be used, as well as any other adhesion material known in the art.

One acceptable location for adhesive dots 26 is in the black matrix region 25. The black matrix region 25 is the region where there is no cathode 13 or phosphor dot. In these black matrix sites 25, the spacer support structures 18 do not distort the display image.

In the illustrative example, the slices 29 are disposed all about the display face 16 or baseplate 21, but the spacer support structures or micro-pillars 18 are formed only at the sites of the adhesive dots 26. The spacer support structures 18 which contact the adhesive dots 26, remain on the display face or baseplate 21. The remaining spacer support structures 18 are removed by subsequent processing. FIG. 5 shows the manner in which the tiles 29 are placed in contact

with the predetermined adhesive dots 26 on the black matrix region 25 of the faceplate 16 or in a location corresponding to the black matrix region 25 along the baseplate 21. The display face 16 or baseplate 21, with slices 29 disposed thereon, is forced against its complementary display surface to enhance adhesion and perpendicular arrangement of the spacer support structures 18 to the display face 16 or baseplate 21.

The glass fibers 18A, 18B, which do not contact an adhesive dots 26, are physically dislodged when the binder or etchable glass strands between the glass fibers 18A, 18B are dissolved, thereby leaving a distribution of contiguous high aspect ratio spacer support structures 18. Since the fibers 18A, 18B are chosen for selective etchability, the etchable strands of glass fibers 18B are removed by applying acid, for example, hydrochloric acid or aqueous hydrofluoric acid. This results in glass spacer support structures 18 in predetermined locations that protrude substantially perpendicular from the display face 16 or baseplate 21, as shown in FIGS. 6A–C.

The selective placement and adhesion of contiguous glass spacer support structures 18, according to the preferred embodiment of the invention, results in a rail structure or I-beam structure, as illustrated in FIGS. 6B and 6C, respectively. The rail or I-beam support structures can be either continuous or discontinuous depending upon the pattern of the glass fibers in the boule 28.

As the spacer support structure 18 is formed from glass fibers 18A, 18B arranged contiguously, a pattern is formed by placing a non-etchable glass strand or fiber 18A proximate an etchable glass strand or fiber 18B, as shown in FIG. 2A. When the tile 29 is exposed to an etchant, the etchable glass strands or fibers 18B are removed, thereby producing a discontinuity in the line of contiguous fibers 18A, 18B. Hence, a pattern is created using contiguous fibers 18A, 18B separated by discontinuities or spaces which result from the removal of the etchable fibers 18B.

In addition to the discontinuities which may result from the selected pattern (e.g., a cross or T-shaped structure), there may be slight discontinuities as a result of the manufacturing process. In such a case, the discontinuity, or break in the line of contiguous fibers, results not from intentional patterning, but rather from a fiber dislodging occurrence in the manufacturing environment.

Since the bending moment of the spacer is dependent on the cross-sectional area, the process of the present invention allows for an increase in the lateral dimension, without a corresponding increase in total surface area.

While the particular process, as herein shown and disclosed in detail, is fully capable of obtaining the objects and advantages herein before stated, it is to be understood that it is merely illustrative of embodiments of the invention, and that no limitations are intended to the details of the construction or the design herein shown, other than as described in the appended claims.

One having ordinary skill in the art will realize that, even though a field emission display was used as an illustrative example, the process is equally applicable to other vacuum displays (such as gas discharge (plasma) and flat vacuum fluorescent displays), and other devices requiring physical supports in an evacuated cavity.

What is claimed is:

1. A method for fabricating a spacer support structure for a flat panel display, the method comprising:  
forming a plurality of fibers each having a rectangular cross-section, said plurality of fibers including a first

group of etchable fibers and a second group of non-etchable fibers; and arranging said first group and said second group of said plurality of fibers so that at least two fibers in said second group are contiguous.

2. The method of claim 1, wherein said arranging comprises arranging said first group and said second group of said plurality of fibers to form a unit cell so that each of said plurality of fibers includes substantially parallel axes.

3. The method of claim 2, wherein said arranging comprises arranging a plurality of unit cells to form a boule so that each of said plurality of unit cells includes substantially parallel axes.

4. The method of claim 3, further comprising slicing said boule into a plurality of slices.

5. The method of claim 4, further comprising adhering at least a portion of said slices to a portion of a surface of the flat panel display.

6. The method of claim 5, further comprising selectively removing said etchable fibers from said slices to form at least one of said spacer support structure, said second group of fibers forming said spacer support structure.

7. The method of claim 1, wherein said arranging comprises selectively arranging said first group and said second group contiguously with parallel axes to form a boule.

8. The method of claim 7, wherein said selectively arranging comprises forming said boule to include a substantially rectangular cross-section.

9. The method of claim 1, wherein said arranging comprises selectively arranging said first group and said second group of said plurality of fibers so that said first group is etchable with respect to said second group.

10. The method of claim 9, further comprising selectively etching said first group with respect to said second group to form a predetermined configuration for said spacer support structure.

11. A display device comprising:

a baseplate;  
a faceplate located opposite said baseplate and in parallel relation thereto; and  
a series of spacer support structures disposed between and connecting said baseplate and said faceplate, said spacer support structures comprising a plurality of fibers each arranged contiguously and substantially parallel thereto, said plurality of fibers each having a rectangular cross-section and arranged in substantially parallel rows and columns.

12. The device of claim 11, wherein said spacer support structures are longitudinally disposed perpendicularly to said baseplate and said faceplate.

13. The device of claim 11, wherein said spacer support structures are longitudinally disposed in parallel relation to said baseplate and said faceplate.

14. The device of claim 11, wherein said spacer support structures comprise at least one of posts, rails, T-shaped structures, and I-beam structures.

15. The device of claim 14, wherein said rails include cross-pieces disposed at substantially right angles thereto.

16. The device of claim 14, wherein said posts exhibit a rectangular cross-section.

17. The device of claim 11, further comprising pixels arranged in rows and columns, said series of spacer support structures being disposed between said pixels.

18. The device of claim 17, wherein said series of spacer support structures is discontinuous.

19. The device of claim 11, further comprising a black matrix disposed on said faceplate, said series of spacer support structures being disposed in said black matrix.

20. The device of claim 11, wherein said series of spacer support structures comprises potash rubidium lead.

21. The device of claim 11, wherein said series of spacer support structures includes a highly resistive coating.

22. A spacer support structure useful in a display device, the spacer support structure comprising:

a plurality of fibers each arranged contiguously and substantially parallel thereto, said plurality of fibers each having a rectangular cross-section and arranged in substantially parallel rows and columns.

23. The spacer support structure of claim 22, wherein said plurality of fibers comprises at least one of a post, a rail, a T-shaped structure, and an I-shaped structure.

24. The spacer support structure of claim 23, wherein said rail includes at least one cross-piece disposed at substantially right angles thereto.

25. The spacer support structure of claim 23, wherein said rail comprises contiguous fiber widths of said plurality of fibers that comprise a length of said rail.

26. The spacer support structure of claim 23, wherein said rail is discontinuous.

27. The spacer support structure of claim 22, wherein said plurality of fibers comprises potash rubidium lead.

28. The spacer support structure of claim 22, wherein said plurality of fibers comprises glass fibers.

29. The spacer support structure of claim 22, wherein said plurality of fibers is collectively arranged to exhibit a rectangular cross-section.

30. The spacer support structure of claim 22, wherein said plurality of fibers each include a rectangular cross-section.

31. A process for fabricating field emission displays, comprising:

forming a baseplate comprising a plurality of micro-cathodes;

forming a faceplate having phosphors disposed thereon; forming a plurality of tiles comprising etchable fibers and nonetchable fibers;

forming said etchable fibers and said nonetchable fibers so that at least two fibers of said nonetchable fibers are contiguous; and

arranging said plurality of tiles on said baseplate.

32. The process of claim 31, wherein said forming said plurality of tiles comprises forming said plurality of tiles to exhibit a substantially rectangular cross-section.

33. The process of claim 31, further comprising selectively removing said etchable fibers to form spacer support structures.

34. The process of claim 33, wherein said selectively removing comprises forming said spacer support structures as posts, rails, I-shaped structures and T-shaped structures.

35. The process of claim 34, wherein said forming comprises forming cross-pieces disposed at substantially right angles to said rails.

36. The process of claim 31, wherein said arranging comprises arranging said tiles contiguously.

37. The process of claim 31, wherein said arranging comprises arranging said nonetchable fibers substantially contiguously.

38. A method for arranging fibers, comprising:

shaping the fibers into strands, each strand having a first rectangular cross-section;

stacking said strands to be substantially parallel and contiguous to form a unit cell, said unit cell having a second rectangular cross-section; and

arranging a plurality of said unit cells to be substantially parallel and contiguous into a boule of said fibers, said boule of said fibers having a third rectangular cross-section.

**39.** The method of claim **38**, further comprising drawing said boule of said fibers to decrease said boule third rectangular cross-section and to increase a length of said boule.

**40.** The method of claim **38**, further comprising slicing said boule of said fibers parallel to said third rectangular cross-section to form tiles of said fibers.

**41.** The method of claim **40**, further comprising placing said tiles of said fibers contiguously about a substrate.

**42.** The method of claim **38**, wherein said stacking of said strands comprises selectively arranging a first group of etchable fibers and a second group of nonetchable fibers.

**43.** The method of claim **42**, further comprising selectively etching said first group of etchable fibers with respect to said second group of nonetchable fibers.

**44.** The method of claim **42**, wherein said selectively arranging comprises arranging said first group of etchable fibers and said second group of nonetchable fibers into a first predetermined pattern in said unit cell.

**45.** The method of claim **44**, wherein said selectively arranging comprises arranging further said plurality of unit

cells into a second pattern, said second pattern built from said plurality of unit cells and said first predetermined pattern thereof.

**46.** The method of claim **45**, further comprising slicing said boule of said fibers to form tiles and placing said tiles on a substrate to form a third predetermined pattern, said third predetermined pattern built from said tiles and said second pattern therein.

**47.** The method of claim **46**, further comprising selectively removing said first group of etchable fibers with respect to said second group of nonetchable fibers to form a shape from said third predetermined pattern.

**48.** The method of claim **47**, wherein said selectively removing to form said shape comprises forming at least one of a post, a rail, an I-shaped structure, and a T-shaped structure.

\* \* \* \* \*

UNITED STATES PATENT AND TRADEMARK OFFICE  
**CERTIFICATE OF CORRECTION**

PATENT NO. : 6,280,274 B1  
DATED : August 28, 2001  
INVENTOR(S) : James J. Hofmann and Jason B. Elledge

Page 1 of 1

It is certified that error appears in the above-identified patent and that said Letters Patent is hereby corrected as shown below:

Column 4,

Line 26, change "over" to -- thereover --

Column 6,

Line 9, after "contact" delete "an"

Line 25, after "respectively." insert -- The thickness of the slice, FIG. 2C will determine whether the cross-section of the rails, etc., is rectangular or square --

Signed and Sealed this

Eighth Day of June, 2004

A handwritten signature in black ink, appearing to read "Jon W. Dudas", is placed on a dotted rectangular background.

JON W. DUDAS  
*Acting Director of the United States Patent and Trademark Office*